

## UNITED STATES PATENT OFFICE

CYRIL J. STAUD AND RUSSEL H. VAN DYKE, OF ROCHESTER, NEW YORK, ASSIGNEES TO  
EASTMAN KODAK COMPANY, OF ROCHESTER, NEW YORK, A CORPORATION OF NEW  
YORK

## PREPARATION OF ACETONE-SOLUBLE FIBROUS NITROACRYLATE

No Drawing.

Application filed December 31, 1930. Serial No. 505,967.

Our invention relates to the production of an acetone-soluble fibrous cellulose nitroacrylate by treating a cellulosic material with a fatty acid anhydride and a liquid oxide of nitrogen in an organic liquid which is a non-solvent (such as carbon tetrachloride), for the cellulose esters which may be present in the reaction mass.

The processes usually employed in the commercial manufacture of cellulose acetate produce a chloroform soluble product which is soluble in the acetylating bath. To render this product soluble in acetone, it may be held for a sufficient period of time in the reaction bath until the desired solubility is attained. Generally, however, some chemical is added to the esterifying bath to destroy the action of the acetic anhydride which may be present therein and to likewise hydrolyze the cellulose acetate. There are a great number of processes for effecting this result.

Manufacturers of cellulose acetate have realized for some time that if a commercial process could be devised to prepare cellulose acetate in the fibrous form and soluble in acetone, considerable economy in the cost of producing this ester would result. In the patents and literature there are processes described for the hydrolysis of chloroform soluble fibrous cellulose acetate, but none of them have proven to be sufficiently economical nor result in a product of sufficiently good quality for commercial application.

An object of the present invention is to provide a process for obtaining fibrous cellulose nitroacetate, soluble in acetone. Another object of the invention is to provide a process of producing this acetone-soluble fibrous cellulose nitroacrylate by one acylation operation without the necessity of hydrolysis. Processes heretofore carried out have involved first either acetylating the cellulose and then nitrating it, or acetylating cellulose nitrate. However, there have been some processes which permitted of a simultaneous acetylation and nitration of cellulose, but none of these have contemplated the use of the effective nitrating agent which comes within the realm of our invention.

We have now found that fibrous cellulose nitroacrylate directly soluble in acetone may be prepared by the use of a liquid oxide of nitrogen in a suitable solvent. The time of acylation, for instance acetylation, may be four hours or even less. However, it has

been found that if the acetylation is allowed to run for 24 hours or even longer improved solubility results. The product is in excellent fibrous form without any lumps or matting together, and gives a clear viscous solution in acetone.

The following examples illustrative of this invention apply to the preparation of acetone-soluble fibrous nitro-acetate.

## Example I

About 50 grams of cotton linters were treated with about 350 grams of glacial acetic acid and 2 c.c. of 1:3 mixed catalyst (sulphuric and phosphoric acids respectively) at room temperature for 14-20 hours. This mixture may then be pressed off to a weight of about 150 grams and cooled down to about 20-25° C. To this pressed mass was added a mixture consisting of about 120 c.c. of 95% acetic anhydride made up to about 450 c.c. with carbon tetrachloride. Before mixing with the anhydride, about 10 c.c. of liquid nitrogen dioxide was added to the carbon tetrachloride. These added materials were mixed thoroughly with the pretreated linters and the temperature of the bath was brought up to 35-50° C., taking about 2 hours, and the mixture was held at this temperature until complete acetylation had taken place. This can easily be completed in 3-5 hours. However, it is preferred that the operation be continued for a longer time. The fibrous cellulose nitrate acetate thus produced was found to be soluble in acetone.

## Example II

About 50 grams of cotton linters were treated with a mixture of about 350 grams of glacial acetic acid and 2 c.c. of 1:3 mixed catalyst at room temperature, as in the previous example. After this pre-treatment the acid is drained off and the linters may be washed two or three times with carbon tetrachloride and allowed to drain. The remaining mass consisted approximately of the following:

|                      | Grams |
|----------------------|-------|
| Cellulose            | 50    |
| Acetic acid          | 98    |
| Carbon tetrachloride | 380   |

The mass was cooled and about 120 c.c. of 95% acetic anhydride was added. This was immediately followed by addition of about 100 c.c. of carbon tetrachloride containing ap-

proximately 10 c.c. of liquid  $\text{NO}_2$  and the whole was thoroughly mixed. The temperature was raised to from 35-50° C., as in Example I, and held at this temperature until complete acetylation had taken place. The fibrous cellulose nitrate acetate produced was found to be soluble in acetone.

One feature of novelty of this invention is the simultaneous fibrous nitration and acetylation of cellulose with a liquid oxide of nitrogen used as the nitrating agent. Although  $\text{NO}_2$ , or  $\text{N}_2\text{O}_4$  are the preferred nitrating agents,  $\text{N}_2\text{O}_3$  or  $\text{N}_2\text{O}_5$  are also satisfactory for this process. It is to be understood that other fatty acids and fatty acid anhydrides may be used instead of the acetic compounds to produce the corresponding fibrous cellulose nitroacrylate. Thus, by the use of butyric acid, or acetic acid, and butyric anhydride, instead of the acetic anhydride, a fibrous cellulose nitro-acetate-butyrate or cellulose nitro-butyrate may be formed.

It is to be understood that other acetylation catalysts may be used instead of the phosphoric-sulphuric mixture. As various acetylation catalysts are well known in the art, enumeration of them is believed unnecessary. Also, in place of carbon tetrachloride, other organic solvents of like nature may be used in this acetylation such as carbon bi-sulphide, trichloroethylene, petroleum distillate, toluol and the like.

It is also to be noted that we may either press off or wash out the pretreating acid from the cellulose prior to acetylation and nitration. Obviously any known method of pressing may be employed and numerous solvents for acetic acid may be used to wash it out of the cellulose. The requirement is merely that the acetic acid present be reduced to a reasonably small amount so that the acylate produced will be retained in the fibrous form by the non-solvent organic liquid added.

What we now claim as our invention and desire to secure by Letters Patent of the United States is:

1. A process of making a fibrous cellulose nitrate-acrylate which comprises treating cellulose with a fatty acid anhydride and a liquid oxide of nitrogen having a boiling point greater than 0° C. in an organic liquid in which the cellulose ester is insoluble.

2. A process of making a fibrous cellulose nitrate-acrylate which comprises treating cellulose with a fatty acid anhydride and a liquid oxide of nitrogen having a boiling point greater than 0° C. in carbon tetrachloride.

3. A process of making a fibrous cellulose nitrate-acetate which comprises treating cel-

lulose with acetic anhydride and a liquid oxide of nitrogen having a boiling point greater than 0° C. in an organic liquid which is a non-solvent for cellulose nitrate-acetate.

4. A process of making a fibrous cellulose nitrate-acetate which comprises treating cellulose with acetic anhydride and a liquid oxide of nitrogen having a boiling point greater than 0° C. in a relatively large amount of an organic liquid which is a non-solvent for cellulose nitrate-acetate.

5. A process of making a fibrous cellulose nitrate-acrylate in a liquid bath which comprises treating cellulose with a fatty acid anhydride and a nitrating agent selected from the group consisting of  $\text{NO}_2$ ,  $\text{N}_2\text{O}_4$ ,  $\text{N}_2\text{O}_3$  and  $\text{N}_2\text{O}_5$  in an organic liquid in which the cellulose ester is insoluble.

6. A process of making fibrous cellulose nitrate-acetate which comprises treating cellulose with acetic anhydride and a liquid nitrating agent selected from the group consisting of  $\text{NO}_2$ ,  $\text{N}_2\text{O}_4$ ,  $\text{N}_2\text{O}_3$  and  $\text{N}_2\text{O}_5$  in an organic liquid which is a non-solvent for cellulose nitrate-acetate.

7. A process of making a fibrous cellulose nitrate-acrylate which comprises treating cellulose with a fatty acid anhydride and liquid  $\text{NO}_2$  in an organic liquid in which the cellulose ester is insoluble.

8. A process of making a fibrous cellulose nitrate-acrylate which comprises treating cellulose with a fatty acid anhydride and liquid  $\text{NO}_2$  in carbon tetrachloride.

9. A process of making a fibrous cellulose nitrate-acetate which comprises treating cellulose with acetic anhydride and liquid  $\text{NO}_2$  in an organic liquid which is a non-solvent for cellulose nitrate-acetate.

10. A process of making a fibrous cellulose nitrate-acetate which comprises treating cellulose with acetic anhydride and liquid  $\text{NO}_2$  in a relatively large amount of an organic liquid which is a non-solvent for cellulose nitrate-acetate.

11. A process of making a fibrous cellulose nitrate-acetate which comprises treating cellulose with acetic anhydride and liquid  $\text{NO}_2$  in carbon tetrachloride.

12. A process of making a fibrous cellulose nitrate-acetate which comprises treating cellulose with acetic anhydride and liquid  $\text{NO}_2$  in an amount of carbon tetrachloride more than six times the weight of the cellulose.

13. A process of making a fibrous cellulose nitrate-butyrate which comprises treating cellulose with butyric anhydride and liquid  $\text{NO}_2$  in carbon tetrachloride.

Signed at Rochester, New York.

RUSSEL H. VAN DYKE.  
CYRIL J. STAUD.